

## UNITED STATES PATENT OFFICE

PERCY ADAMSON, OF RYE, NEW YORK

## ELASTIC YARN

No Drawing.

Application filed June 11, 1931. Serial No. 543,737.

This invention relates to elastic yarn suitable for use in the manufacture of various textile fabrics and articles.

This application is a continuation in part of my prior application Serial No. 470,400, filed July 24, 1930.

Elastic yarns as heretofore marketed have been relatively large and unsuitable for the manufacture of knit articles. They have been made from cores of vulcanized rubber composition wound with one or more yarns and in one or more layers. The cores were of relatively large size cut square in cross section. The fibrous covering yarns have been relatively coarse and have substantially augmented the dimensions of the core. Because of these factors and because also of the lack of uniformity in the built-in elongation of the core and of the covering operations, the old elastic yarns were not employed in knitting machines, especially those of fine gauge. Such old elastic yarns were used largely in the manufacture of woven fabrics such as elastic straps for girdles and for stocking supports and of such articles as garters, bandages, and the like. Furthermore, the old elastic yarns, as heretofore utilized in making articles, generally, if not invariably, imparted a capacity to stretch in one direction only. In other words, they were practically only used for making articles which resisted a one-direction pull or which exerted a constrictive force in one direction.

The present invention aims to provide a new and useful type of elastic yarn which has characteristics adapting it to be utilized in knitting machines of fine gauge—as fine or finer than cylindrical knitting machines of a diameter of  $3\frac{1}{2}$  inches having 176 needles.

With it a large variety of articles having new

and improved qualities long desired in the art may be manufactured. The capacity of the elastic yarn for knitting in modern fine gauge knitting machines at high speed enables it to be utilized with existing equipment, without substantially increased labor or handling costs; and without great reduction, if any, in the speed of the machines. It enables articles to be fabricated with a capacity to stretch or yield in any direction rather than merely in one direction whereby the grip of the article on the body or portions of the body is distributed and made comfortable to the wearer without sacrifice of holding or sustaining capacity.

With the elastic yarn of the present invention it is now practical to manufacture hosiery for men, women, and children of fine gauge with an integral garter-like portion for effectively sustaining the hose in a comfortable manner, to manufacture corsets, foundation garments, brassières, bathing suits, surgical bandages, etc., all with a capacity to enhance the lines of the human figure in a comfortable manner and with a position-retaining capacity not heretofore attained, and to manufacture so-called surgical stockings which are comfortable and efficacious to those afflicted with varicose veins, etc. Many other articles with superior qualities, as those skilled in the art will appreciate, may be made of this new elastic yarn. It has already aroused great interest among garment manufacturers, particularly the hosiery and underwear trade, and great activity has followed its disclosure.

According to my invention, a core of any suitable elastic material uniformly elongated is covered with relatively inelastic fibrous material holding it stretched. In the

manufacture of a particular elastic yarn the elongation uniformly given the yarn is so adjusted with respect to the covering yarn that the finished yarn has a predetermined and limited capacity to stretch. During the covering operation whatever tension is applied to the core should be applied uniformly and evenly throughout the covering operation. The capacity to stretch of the finished 5 elastic yarn may be anything desired but preferably, at least for use on fine gauge knitting machines, should be in the neighborhood of 150%, i. e., 1" of normal elastic yarn should stretch to 2 1/2". To obtain the 10 best speed in the operation of the finest gauges of knitting machines the capacity to stretch is desirably made somewhat less and more in the neighborhood of 100%. Of course the stretching capacity of the elastic yarn 15 should also be suited to the use to which it is put, and may vary from those percentages which are illustrative.

For the core of the elastic yarn any vulcanized rubber composition of a high grade 20 is suitable but it is preferred to utilize rubber of a grainless character such as that obtained by suitably compounding rubber latex and fashioning it into fine rubber thread without sharp corners and uniform in cross section, 25 the optimum being circular and of a gauge suitable for the use in view. For most purposes, the core, at least when made of rubber derived from rubber latex, should be of a thickness between .0133 and .0080 of an inch, 30 in its normal or relaxed condition, but both larger and smaller cores may be utilized. Such fine gauge cores, at least when made of vulcanized rubber composition, may readily be produced in any desired lengths in the manner 35 disclosed in the prior patent to Hopkinson and Gibbons No. 1,545,257 granted July 7, 1925. It is to be understood however that the invention is not limited, in its broadest aspects at least, to the use of cores made 40 by following such patent and that cores for use in the manufacture of the elastic yarn of this invention may be made in any convenient manner, shape, and size, and from any suitable materials approximating in 45 qualities high rubber content stocks which possess good stretch and return characteristics. Cores made from concentrated (60%) rubber latex suitably compounded to resist 50 aging and to permit vulcanization at moderately low temperatures are preferable, particularly when of circular cross section by the method disclosed in said patent because they may be made readily without irregularities or 55 jagged surfaces commonly present in cut threads, and with less likelihood of breaking or parting under successive stretching and relaxing treatments in service. The importance of this feature of construction in 60 such fine elastic yarns as are required for 65

most knit articles will be apparent. With some advantage the rubber cores may be made from rubber latex in other convenient ways as rubber derived from latex is grainless and possesses greater resistance to tearing. The 70 cores however may be made of vulcanized rubber composition or any other suitable material that is capable of regaining its normal length after elongation in the manner of rubber. 75

The relatively inelastic fibrous covering may be applied in any suitable and convenient manner as those skilled in the art will understand. Yarns of cotton, linen, flax, silk, rayon, wool, or the like may be employed, 80 and while they may be braided about the core, it is preferred to use right and left helical windings of small and either alike or different pitch, the relative pitch of the windings being selected with due consideration to the size and nature of the materials being wound in order to obtain an approximately balanced elastic yarn, relatively free from a tendency to kink. The helical windings may be of like or of different materials 85 and either may consist of one or more ends of yarn or plied yarn depending upon the characteristics it is desired to build into the elastic yarn to meet the requirements of the 90 service to which it is to be subjected in the article manufactured therefrom. 95

In general, in manufacturing the elastic yarn of this invention, the core of elastic material while being wound and substantially 100 completely covered, should be elongated uniformly, the more uniform the better. While the elongation or stretch may vary for different elastic yarns, it should not vary in any one particular yarn in order to obtain a product which in knitting on a machine will not only make stitches without dropping them but will make them uniformly and thereby 105 yield an even knit fabric. The yarn selected should be relatively small in cross section. If more than one end is employed, in other words, if a ribbon of two or more yarns in parallelism is used, the pitch of the helical winding will of course be substantially greater than when a single similar yarn is being wound. 110

Structural characteristics of specimens of elastic yarn are given in Table I hereinafter. 115 In considering the data therein it is to be noted that much of it was compiled from a yard length, or from a fraction of a pound, of the elastic yarn, and consequently, any slight error in measurement thereof may have 120 been multiplied. Obviously the flexible and yielding nature of the core of elastic material and of the covering yarn, which together 125 constitute the elastic yarn, renders its analysis difficult and meticulous accuracy impossible. 130

The table following is therefore to be taken as illustrative.

TABLE I.—Analyses of actual samples

| Designation                                                               | A              | B              | C              | D                  | 70 |
|---------------------------------------------------------------------------|----------------|----------------|----------------|--------------------|----|
| 1. Gauge of circular rubber core—normal condition.                        | .019           | .013+          | .01            | .008               |    |
| 2. Elongation of rubber core during winding—approximately.                | 340%           | 280%           | 270%           | 370%               |    |
| 3. Yards per pound—normal condition.                                      | 2,875          | 4,220          | 5,610          | 15,000             |    |
| 4. Elongation—increase over normal length on stretching to limit.         | 115%           | 125%           | 120%           | 170%               |    |
| 5. Material of outside cover.                                             | 5-100/1 cotton | 3-100/1 cotton | 3-100/1 cotton | 1-2 ply 13/15 silk |    |
| 6. Material of inside cover.                                              | 1-140/2 cotton | 1-120/2 cotton | 1-120/2 cotton | 1-2 ply 13/15 silk | 75 |
| 7. Wraps per inch—outside cover.                                          | 45.2 L         | 54.8 L         | 61.6 L         | 122.2 L.           |    |
| 8. Wraps per inch—inside cover.                                           | 52.0 R         | 58.0 R         | 72.9 R         | 121.6 R            |    |
| 9. In one yard of normal elastic yarn, the inches of bare rubber—relaxed. | 15.9"          | 20.2"          | 15.9"          | 18"                |    |
| 10. In one yard of normal elastic yarn, the weight in grams of—           |                |                |                |                    |    |
| (a) Bare rubber.                                                          | .073           | .045           | .018           | .014               |    |
| (b) Both rubber and covers.                                               | .1625          | .108           | .081           | .035               | 80 |
| 11. Per cent by weight of rubber core.                                    | 44.9%          | 41.9%          | 22.2%          | 40%                |    |
| 12. Per cent by weight of outside cover.                                  | 44.0%          | 39.1%          | 54.3%          | 28.6%              |    |
| 13. Per cent by weight of inside cover.                                   | 11.1%          | 19.0%          | 23.5%          | 31.4%              |    |
| 14. Yardage of 1 pound of bare rubber core—relaxed.                       | 2,740          | 5,670          | 11,100         | 16,200             |    |
| 15. Yardage of relaxed bare rubber in 1 pound elastic yarn.               | 1,260          | 2,380          | 2,480          | 7,300              |    |
| 16. Gauge in inches of elastic yarn (product).                            | .017+          | .015           | .015           | .006               |    |

20 The gauge of the elastic yarn (item 16) was measured by an automatic micrometer which pressed upon four adjacent yarns with a uniform constant pressure of 6 ounces. The four threads held at each end about six inches apart were placed under the presser foot which was  $\frac{3}{8}$  of an inch in diameter and the reading recorded. The presser foot was

core, if it be of rubber, of the amount of talc or other dusting material picked up by the core of elastic material incident to its manufacture and manipulation, of the elongation of the core during its winding, of the pitch of the windings of the cover, and of the covering yarns themselves. With these cautions the specifications of Table II are now given.

TABLE II.—Specifications

| Designation                                                             | E              | F              | G              | H                  | 95  |
|-------------------------------------------------------------------------|----------------|----------------|----------------|--------------------|-----|
| 1. Gauge of circular rubber core—normal condition.                      | .020           | .013+          | .010           | .003+              |     |
| 2. Elongation of rubber core during winding approximately.              | 340%           | 280%           | 270%           | 370%               |     |
| 3. Yards per pound—normal condition.                                    | 3,140          | 4,560          | 5,420          | 14,000             |     |
| 4. Elongation—increase over normal length on stretching to limit.       | 120%           | 120%           | 120%           | 170%               | 100 |
| 5. Material of outside cover.                                           | 3-100/3 cotton | 3-100/1 cotton | 3-100/1 cotton | 1-2 ply 13/15 silk |     |
| 6. Material of inside cover.                                            | 1-120/2 cotton | 1-120/2 cotton | 1-120/2 cotton | 1-2 ply 13/15 silk |     |
| 7. Wraps per inch—outside cover.                                        | 45 L           | 55 L           | 62 L           | 122 L.             |     |
| 8. Wraps per inch—inside cover.                                         | 55 R           | 65 R           | 72 R           | 122 R.             |     |
| 9. In 1 yard of normal elastic yarn, the inches of bare rubber—relaxed. | 16"            | 16"            | 16"            | 18"                |     |
| 10. In 1 yard of normal elastic yarn, the weight in grams of—           |                |                |                |                    |     |
| (a) Bare rubber.                                                        | .0300          | .0354          | .0198          | .014               |     |
| (b) Both rubber and covers.                                             | .1445          | .0993          | .0337          | .035               |     |
| 11. Per cent by weight of rubber core.                                  | 56%            | 35.7%          | 23.6%          | 40%                |     |
| 12. Per cent by weight of outside cover.                                | 29.5%          | 42.9%          | 51.0%          | 28.6%              |     |
| 13. Per cent by weight of inside cover.                                 | 14.5%          | 21.4%          | 25.4%          | 31.4%              |     |
| 14. Yardage of 1 pound of bare rubber core—relaxed.                     | 2,500          | 5,700          | 10,200         | 16,000             |     |
| 15. Yardage of relaxed bare rubber in 1 pound elastic yarn.             | 1,400          | 2,030          | 2,410          | 7,200              |     |
| 16. Gauge in inches of elastic yarn (product).                          | .019           | .017           | .015           | .008               | 110 |

50 raised a fraction of an inch from the base and allowed to snap back on the elastic yarns. The pressure spring in this micrometer was equivalent to that obtained by six ounces dead weight dropped a fraction of an inch in vertical position.

55 The above analyses are but a few of many that have been made. From all of the data accumulated specifications have been formulated for guidance in the production of yarns ordered. Three such specifications for elastic yarns with cotton coverings are given in 60 subsequent Table II under the columns headed E, F and G, and one for a silk covering in the column headed H. It is not to be expected that these specifications will be exactly realized in the manufacture of any 65 particular elastic yarn because of the many

It will of course be understood that the specifications of the foregoing tables are not given with any intention to limit the invention more than is required by the scope of the prior art. Obviously the relative size and materials of both the core and the covering yarns may be varied to meet requirements, likewise also the elongation of the core during winding, and the pitch of the windings or the wraps per inch. As before indicated, the capacity of the elastic yarn to stretch may be varied as desired but it is preferable, at least for knitting on fine gauge machines, to keep such capacity down to the neighborhood of 150% or down to 100%.

65 From the foregoing the nature of the invention will be apparent to one skilled in the art. The elastic yarn may be employed in knitting machines in the manufacture of all

or part of knitted articles, and either as a substitute for the ordinary non-elastic fibrous knitting yarns, or jointly therewith in so-called "plating". The elastic yarn may also be used on sewing machines for stitching purposes. It may also be used as a substitute for the old elastic yarns where it is desired to obtain a finer product. Woven or knitted into bandages the universal elasticity of the fabric enables an end of the bandage to be tucked under a convolution and anchored by its own inherent gripping properties. Incorporated in articles of wearing apparel such as corsets, brassières, or bathing suits, desirable figure-enhancing effects may be attained. Golf knickers and socks may be improved by its use. Great improvements in many old articles of manufacture and in many new articles are attending its introduction and disclosure. A few courses of elastic yarn incorporated in women's stockings immediately above the knee will minimize runs. In such cases, and generally in knitting, it is advisable to relieve the elastic yarn of tension so that when the garment is completed the portion thereof constituted by the elastic yarn, will not contract or narrow in such way as to objectionably detract from its appearance and this may be done by leading the yarn directly from the source of supply to the knitting needles instead of through the usual tensioning devices.

The invention is not intended to be limited beyond the extent required by the scope of the prior art and all changes and variations as may be made within it are intended to be comprehended. Reference should therefore be made to the accompanying claims for an understanding of the scope of the invention. In the claims the term elastic material is used to comprehend rubber compositions and any materials equivalent thereto for the purposes of this invention.

Having thus described my invention, what I claim and desire to protect by Letters Patent is:

1. An elastic yarn capable of being knitted in a knitting machine and having a core of elastic material under tension, and a covering of relatively inelastic fibrous material holding the core elongated, said elastic yarn being limited to a predetermined and substantially uniform degree in its capacity to stretch, a pound of said elastic yarn in its normal condition having a total length of more than 2800 yards.

2. An elastic yarn capable of being knitted in a knitting machine and having a core of elastic material under tension, and a covering of relatively inelastic fibrous material holding the core elongated, said elastic yarn being limited to a predetermined and relatively uniform degree in its capacity to stretch, a pound of said core of elastic mate-

rial in a normal unstretched condition alone measuring at least 5000 yards.

3. An elastic yarn capable of being knitted in a knitting machine and having a core of elastic material under tension, and a covering of relatively inelastic fibrous material holding the core elongated, said elastic yarn being limited to a predetermined and substantially uniform degree in its capacity to stretch, a pound of said elastic yarn in its normal condition containing a core of elastic material, which core, when freed of said covering and relaxed, measures in excess of 1000 yards.

4. An elastic yarn capable of being knitted in a knitting machine and having a core of elastic material under tension, and a covering of relatively inelastic fibrous material holding the core elongated, said elastic yarn being limited to a predetermined and uniform degree in its capacity to stretch, the greatest dimension of an average cross section of said elastic yarn being less than .025 of an inch.

5. An elastic yarn capable of being knitted in a fine gauge knitting machine and having a core of vulcanized rubber composition under tension, right and left helical windings of yarn covering said core and holding it elongated, said yarn having a predetermined and substantially uniform capacity to stretch, a pound of said elastic yarn in its normal condition having a total length of at least 3600 yards.

6. An elastic yarn capable of being knitted in a fine gauge knitting machine and having a core of vulcanized rubber composition under tension, right and left helical windings of yarn covering said core and holding it elongated, said yarn having a predetermined and substantially uniform capacity to stretch, a pound of said core of elastic material in a normal unstretched condition alone measuring at least 5000 yards.

7. An elastic yarn capable of being knitted in a fine gauge knitting machine and having a core of vulcanized rubber composition under tension, right and left helical windings of yarn covering said core and holding it elongated, said yarn having a predetermined and substantially uniform capacity to stretch, a pound of said elastic yarn in its normal condition containing a core of elastic material, which core, when freed of said right and left helical windings of yarn and relaxed measures more than 1200 yards.

8. An elastic yarn capable of being knitted in a fine gauge knitting machine and having a core of vulcanized rubber composition under tension, right and left helical windings of yarn covering said core and holding it elongated, said yarn having a predetermined and substantially uniform capacity to stretch, the greatest dimension of an average cross section of said elastic yarn not exceeding .021 of an inch.

9. An elastic yarn having a core of vulcanized rubber composition under tension, a plurality of balanced windings of yarn covering said core and holding it elongated, said core when uncovered and relieved of tension being approximately circular in cross section, said elastic yarn having a predetermined and uniform capacity to stretch and to flex in any direction throughout its length, and said elastic yarn having a length of more than 2,000 yards in a pound thereof in a relaxed normal condition.
10. An elastic yarn having a core of vulcanized rubber composition under tension, and right and left helical windings of fibrous yarn holding the core elongated, the capacity of said elastic yarn to stretch and to flex in any direction being uniform throughout its length, the flexibility of said elastic yarn being such as to permit knitting in a fine gauge knitting machine at normal speeds without dropping stitches, and said elastic yarn having a length of more than 2,000 yards in a pound thereof in a relaxed normal condition.
11. An elastic yarn having a core of vulcanized rubber composition under tension, right and left helical windings of fibrous yarn holding the core elongated, the capacity of said elastic yarn to stretch and to flex in any direction being uniform throughout its length, the flexibility of said elastic yarn being such as to permit knitting in a fine gauge knitting machine at normal speeds without dropping stitches, and said core being approximately circular in cross section when freed of said windings and relieved of tension, and said elastic yarn having a length of more than 2,000 yards in a pound thereof in a relaxed normal condition.
12. An elastic yarn having a core of vulcanized rubber composition under tension, right and left helical windings of fibrous yarn holding the core elongated, the capacity of said elastic yarn to stretch and to flex in any direction being uniform throughout its length, the flexibility of said elastic yarn being such as to permit knitting in a fine gauge knitting machine at normal speeds without dropping stitches, said core being approximately circular in cross section when freed of said windings and relieved of tension, and said elastic yarn having an external diameter of less than .021 of an inch.
13. An elastic yarn having a core of vulcanized rubber composition under tension, and a fibrous covering holding said core elongated, said elastic yarn having approximately the characteristics of a non-elastic yarn of approximately the same size and of approximately the same materials as the fibrous covering for the elastic yarn excepting in its stretching characteristics, and said elastic yarn having a length of more than 2,000 yards in a pound thereof in a relaxed normal condition.
14. An elastic yarn having a core of vulcanized rubber composition under tension, and right and left helical windings of yarn covering and holding the core elongated, said core and said windings being of such size and said windings being of such material and so applied as to adapt the elastic yarn for knitting in a fine gauge cylindrical knitting machine of a diameter of 3½ inches having at least 176 needles, or in an equivalent fine gauge knitting machine, and said elastic yarn having a length of more than 2,000 yards in a pound thereof in a relaxed normal condition.
15. An elastic yarn having a core of vulcanized rubber composition under tension, and right and left helical windings of yarn covering and holding said core elongated, the size of said elastic yarn approximating the size of said core of vulcanized rubber composition before it is wound and before it is stretched, and said elastic yarn having a length of more than 2,000 yards in a pound thereof in a relaxed normal condition.
16. An elastic yarn having a core of vulcanized rubber composition under tension, said core being uniform in cross-section and having smooth external surfaces substantially free from corners and irregularities, covering yarn holding said core elongated, said elastic yarn being uniformly stretchable to a predetermined limit, said elastic yarn being uniformly flexible in any direction throughout its extent, and the average cross section of said elastic yarn being less than .021 of an inch.
17. An elastic yarn having a core of vulcanized grainless rubber composition under tension, a covering of relatively inelastic fibrous material holding said core elongated and limiting the capacity of the elastic yarn to stretch to a predetermined degree, the average thickness of said elastic yarn being less than .021 of an inch.
- Signed at New York, county of New York, State of New York, this 10 day of June, 1931.
- PERCY ADAMSON

## DISCLAIMER

1,822,847.—*Percy Adamson, Rye, N. Y.* ELASTIC YARN. Patent dated September 8, 1931. Disclaimer filed March 10, 1939, by the assignee, *United States Rubber Company*.

Hereby enters its disclaimer to that part of the specification and claims enumerated as follows, to wit:

From the specification of said patent all data in column A of Table I and all data in column E of Table II on page 3 thereof, and all reference in such specification to said data; and

Claims 4 and 15; and

From claim 3 of said patent all elastic yarns therein defined save those which have a core, the average thickness of which does not exceed .0133 of an inch in relaxed uncovered condition; and

From each of claims 1, 5, 7, and 8 of said patent all elastic yarns therein defined save those which are capable of being knitted without appreciable reduction of speed of, and without dropping stitches on, knitting machines of fine gauge as fine or finer than cylindrical knitting machines of a diameter of 3½ inches having 176 needles and which yarns are capable of use as a substitute for the ordinary non-elastic fibrous knitting yarns; and

From each of claims 10 and 11 of said patent all elastic yarns therein defined save those which are capable of being knitted on knitting machines of fine gauge as fine or finer than cylindrical knitting machines of a diameter of 3½ inches having 176 needles; and

From claim 13 of said patent all elastic yarns therein defined save those which are capable of being knitted without appreciable reduction of speed of, and without dropping stitches on, knitting machines of fine gauge as fine or finer than cylindrical knitting machines of a diameter of 3½ inches having 176 needles.

[Official Gazette April 4, 1939.]